

## UNITED STATES PATENT OFFICE

COLIN G. FINK, OF NEW YORK, N. Y., ASSIGNOR TO ALLEGHENY STEEL COMPANY, OF BRACKENRIDGE, PENNSYLVANIA, A CORPORATION OF PENNSYLVANIA

## METHOD OF IMPROVING THE RESISTANCE OF ALLOY ARTICLES TO CORROSION

No Drawing. Original application filed November 4, 1927, Serial No. 231,156. Divided and this application filed June 26, 1930. Serial No. 464,112.

This invention relates to a method of improving the resistance of alloy articles to corrosion, and to the products of such method, and is a division of my copending application, 5 Serial No. 231,156 filed November 4, 1927.

By the present method, the resistance of articles made from various corrosion-resistant alloys is very largely improved. The invention further provides a process which 10 may be readily practiced, and by which the improved results are obtained in an economical manner. The invention further provides a means of regenerating or recovering materials used in the processes.

15 According to the present invention, an article made of corrosion-resistant alloy is treated in such a way as to dissolve from the surface the more soluble parts or elements of its surface, so as to leave a surface composed of the more resistant parts or elements of the alloy, and the pores or crystal interspaces are packed or filled with a compound of a metal capable of forming a corrosive-resistant oxid, in such a manner as to stop or retard the 20 progress of corrosion through the pores or crystal interspaces and thereby prevent the undermining of the more resistant parts or elements of the alloy left at the surface.

The invention is applicable generally to 30 the treatment of corrosion-resistant alloys, and particularly to the alloys of iron with chromium and metals related to chromium, such as molybdenum, vanadium, titanium, tungsten, manganese, cobalt and nickel.

35 The invention will be more particularly described with reference to ferro-chromium alloys, and particularly with reference to the so-called low chromium alloys containing, for example, 5 to 15 per cent chromium.

40 In carrying out the process, the more soluble parts of the alloy, the iron-rich constituents of ferro-chromium alloys for example, are removed by an acid which acts strongly upon such soluble parts and less 45 strongly or not at all upon the more resistant parts of the alloy. The common mineral acids can be used, but sulphuric acid is preferred, particularly with ferro-chromium alloys.

50 The packing of the pores or crystal inter-

spaces is effected by a solution containing a compound of a metal which forms a corrosion-resistant oxid. Suitable compounds are soluble compounds of chromium, titanium, vanadium, tungsten, molybdenum, manganese, etc.

The articles are preferably subjected at one immersion to the action of the acid for dissolving the more soluble parts of the alloy and of the compound of the metal for packing 60 the pores or crystal interspaces, the articles being immersed in a solution containing both the acid and the compound of the metal for packing the crystal interspaces.

The treatment is preferably carried out in 65 a hot bath.

It is important and therefore preferable to pickle the articles, so as to obtain a clean surface, prior to treating the articles to the action of the acid for selectively dissolving 70 the surface, and to the compound for packing the crystal interspaces or pores.

A mode of procedure by way of example is as follows:

An article of a resistant alloy, as for example a low-chromium, ferro-chromium alloy tube, is first preferably pickled or cleaned. A suitable pickling solution, for example, would be a solution of zinc chloride and hydrochloric acid.

After the article has been cleaned, it is then placed in a bath of sulphuric acid and chromic acid for selectively dissolving the iron-rich parts of the surface metal and packing or filling the crystal interspaces or pores.

Various concentrations of sulphuric acid and chromic acid may be used; I have found it preferable, however, to regulate the sulphuric acid to approximately 7 per cent sulphuric acid (6 cc. concentrated oleum in 100 cc. water). It is preferable to have the chromic acid somewhat concentrated in the bath, as for example at approximately 60%  $\text{CrO}_3$  (135 grams chromic acid per 100 cc. water). The bath is preferably kept at boiling temperature.

With such a solution containing around 7% sulphuric acid and 60% chromic acid, an improved effect is produced in a comparatively short time. For example, by boiling test-

pieces in such a solution from 40 to 90 minutes the loss in weight when subjected to a salt-spray test at 40° C. for 90 hours is less than can be weighed, the test-pieces showing 5 no signs of corrosion and retaining their bright surface appearance.

The article after treatment according to my process is one which is very much more 10 resistant to corrosion than before treatment, and in the example given, as stated above, samples do not lose perceptibly in weight after being subjected to the salt-spray test at 40° C. for 90 hours. By dissolving the iron-rich constituents out of the surface of 15 the alloy, the article is left with a surface composed of chromium-rich constituents. The undermining of this chromium-rich surface is prevented by the chromic acid compounds which fill or pack the pores and crystal interspaces. The chromic acid is the 20 trioxide of chromium, and eventually converts into the more stable sesqui-oxid  $\text{Cr}_2\text{O}_3$ , or corresponding compounds with iron. The corrosion resistant alloy articles form the subject matter of my companion application filed 25 June 26, 1930, bearing serial number 464,111.

In carrying out the process it has been found that the action of the chromic acid, sulphuric acid solution becomes sluggish 30 when the concentration of the solution reaches approximately 80 grams per liter of iron.

In order to render the solution usable and to recover the valuable constituents of the bath, it is preferable to regenerate as follows:

The sluggish solution is led into a tank containing a hot solution of half sulphuric acid and half water. The heat may be derived from the action of the sulphuric acid and 40 water when added together, or be otherwise supplied. In this solution the chromic acid is precipitated as crystals of  $\text{CrO}_3$ , the iron sulphate not being precipitated immediately from a hot solution. The chromic acid crystals 45 are conveniently removed by filtering, or by centrifuging. The commercial recovery exceeds 90% of the chromic acid present. The recovered chromic acid may be redissolved in making up new solutions or in 50 strengthening solutions.

The sulphuric acid and iron sulphate dissolved or suspended therein may be separated by concentrating the sulphuric acid in an evaporator, for example, the iron sulphate 55 precipitating in the concentrated sulphuric acid solution and settling as a sludge. The supernatant sulphuric acid may be siphoned off or decanted, and used again in the process.

The invention may be carried out in various 60 other modes of procedure than that herein specifically described.

What I claim as new and desire to secure by Letters Patent is:

1. A method of improving the resistance 65 of ferro-alloy articles to corrosion, compris-

ing immersing said articles in a 7% solution of an acid, which is strong as regards the iron-rich parts of the alloy, and of 60% chromium trioxid (chromic acid), and regenerating said solution when the iron content 70 approximates 80 grams per liter.

2. A method of improving the resistance of ferro-alloy articles to corrosion, comprising immersing said articles in a bath containing about 7% sulphuric acid and about 60% 75 chromic acid.

3. A method of improving the resistance of ferro-alloy articles to corrosion, comprising forming a boiling bath containing about 7% sulphuric acid and about 60% chromic acid, 80 immersing said articles in said bath until the surfaces of said articles have had dissolved out of them the iron-rich constituents which are replaced by a corrosion resistant chromium compound. 85

4. A method of improving the resistance of ferro-alloy articles to corrosion comprising treating the surfaces of said articles with a bath of sulphuric acid and chromic acid to dissolve the soluble parts of the surfaces thereof and deposit chromium oxide in place of said dissolved parts, said bath containing 90 7% sulphuric acid and 60% chromic acid.

5. A method of improving the resistance of ferro-alloy articles to corrosion comprising 95 treating the surfaces of said articles with a hot bath of sulphuric acid and chromic acid to dissolve the soluble parts of the surfaces thereof and deposit chromium oxide in place of said dissolved parts, said bath containing 100 7% sulphuric acid and 60% chromic acid.

In testimony whereof, I have hereunto subscribed my name this 21 day of June 1930.

COLIN G. FINK.

105

110

115

120

125

130